

## UNITED STATES PATENT OFFICE

2,104,049

## TREATMENT OF MOTOR FUEL

Jacque C. Morrell, Chicago, Ill., assignor to Universal Oil Products Company, Chicago, Ill., a corporation of Delaware

No Drawing. Application July 29, 1932,  
Serial No. 626,178

9 Claims. (Cl. 44—9)

This invention relates more particularly to the treatment of motor fuels produced in the cracking of various primary tars such as, for example, those produced in the distillation of coals, woods, lignites, oil shales, etc.

More specifically, the invention has reference to a process whereby such low boiling motor fuel fractions are refined and stabilized so that on storage under the influence of light and air there is substantially no deterioration in regard to knock rating or the development of color and gums or other undesirable characteristics.

The types of tars with which the invention is concerned vary in character and composition according to variations in the primary carbonaceous material from which they are produced and also vary with the conditions of distillation, particularly in regard to the pressures, temperatures and rates of heating employed. These primary tars contain varying proportions of the principal hydrocarbon groups, to wit, paraffins, olefins, naphthenes and aromatics, and also contain nitrogen, oxygen and sulphur compounds. In cracking such mixtures, the products obtained will depend upon the relative proportions of the classes of hydrocarbons and hydrocarbon derivatives which are present, the boiling ranges of the different groups and the conditions employed in cracking.

In regard to the products from cracking the nitrogen, oxygen and sulphur derivatives, particularly in the presence of preponderating amounts of hydrocarbons, less information is available but in general it may be assumed that the various groups of derivatives produce lower boiling compounds of the same type although their decomposition is influenced to some extent by the products of the hydrocarbon decomposition reactions.

In one specific embodiment, the invention comprises cracking primary tars containing phenolic compounds under elevated temperatures and pressures to produce low boiling motor fuel fractions, treating said motor fuel fractions with alkalies to remove phenols, separating phenols from the alkali solutions by acidification thereof and returning regulated amounts of the selected fractions of the separated phenols to the treated motor fuel fractions, preferably after first refining the same by further well known treatment such as with sulphuric acid, to inhibit the loss of valuable properties therein during storage under the influence of light and air. The motor fuel fractions may be further treated with dilute acids which are later neutralized with alkali and the

recovered basic materials may then be added to the treated motor fuel in regulated amounts.

Inhibitors are to be distinguished from antiknock agents in that the true antiknock agent modifies the combustion of fuel in an internal combustion engine cylinder but does not necessarily prevent the development of undesirable characteristics under storage. In fact, numerous well defined antiknock agents are themselves unstable in storage and the gasoline to which they are added needs further additions of true inhibitors to stabilize the increased antiknock value produced by the addition of the antiknock agent. Furthermore, it is usually necessary to use much higher percentages of reagents to prevent knocking than is necessary in inhibiting deterioration and depreciation of the gasoline so that it will be seen that in the great majority of cases the action of antiknock agents is distinct from that of true inhibitors such as the phenolic mixtures used in the present invention.

Numerous compounds of a phenolic character have been employed as inhibitors, the ones most generally used being individual chemical compounds produced by synthesis from simpler materials or by tedious and expensive processes which effect their separation from primary tars. The present process is self-contained in that the inhibiting materials are a product of the process so that greater economy is possible than in the use of such materials manufactured by special outside processes. The amount of phenolic fractions possessing inhibiting value which are present in the cracked products from primary tars is usually in excess of that required for properly stabilizing the treated motor fuel so that only relatively small quantities and select fractions of the tar acids extracted by caustic alkalies are necessary to effect the required stabilization of properties. Such fractions may be produced by redistilling the separated tar acids to produce a plurality of overhead cuts which may then be tested to see which cut or blend of cuts is of the greatest value. Such redistillation will also leave behind as a residue any heavy pitchy or tarry materials which would add color to the treated motor fuel even when used in small amounts of the order of 0.05%.

The following examples of results obtainable by the use of the process of the invention on coal, wood and lignite tars, respectively, will serve to show its commercial advantages.

A coal tar derived from Ohio-Indiana bituminous coal by low temperature distillation was

cracked at 100 pounds pressure and 800° F. The analysis of the tar is given in the following table:

|                          |                            |
|--------------------------|----------------------------|
| Sp. Gr.                  | 1.0794                     |
| I. B. P.                 | 240° F.                    |
| 5 Flash                  | 130° F. Cleveland open cup |
| Fire                     | 180° F. Cleveland open cup |
| Furol visc.              | 122° F.                    |
|                          | 70 sec.                    |
| Per cent distilled over  | °F.                        |
| 10                       | 406                        |
| 20                       | 450                        |
| 30                       | 495                        |
| 40                       | 555                        |
| 50                       | 658                        |
| 15                       | 702                        |
| 60                       | 78                         |
| 78                       | 690                        |
| Coke per cent by weight  | 22.0                       |
| Tar acids per cent       | 27.5                       |
| Bases per cent           | 1.55                       |
| 20 Neutral oils per cent | 28.95                      |

This tar yielded, under the conditions stated, 33.9% of motor fuel boiling range fractions containing 35% tar acids or 22% of motor fuel fractions on an acid-free basis. In the present instance, the solution of tar acids was acidified and the acids distilled at atmospheric pressure to produce fractions corresponding to 25° C. boiling ranges beginning at 225° C. These fractions were tried separately upon the acid and alkali refined motor fuel to determine their value as inhibitors and it was found that the use of 0.05% of any of the fractions in the treated gasoline was ample to stabilize and conserve the valuable properties, such as color, low gums and antiknock value. The fraction of highest value in preventing deterioration of the gasoline was found to be that boiling between 250° and 275° C., and the use of this fraction raising the induction period in the oxygen bomb test from 50 minutes to 400 minutes, 40 which is in excess of the ordinarily required 240 minute maximum.

As another example of the use of the process, a wood tar derived from the distillation of Douglas fir was cracked under a pressure of 120 pounds per square inch and a temperature of approximately 775° F. The analysis of the original tar is given in the following table:

Table 2

|                             |                   |
|-----------------------------|-------------------|
| 50 Specific gravity         | 1.061             |
| A. P. I. gravity            | 1.7               |
| Initial boiling point:      |                   |
| °F.                         | 240               |
| °C.                         | 116               |
| 55 Per cent over            | °C.               |
| 10                          | 172               |
| 20                          | 228               |
| 30                          | 263               |
| 40                          | 288               |
| 60                          | 314               |
| 50                          | 332               |
| 60                          | 344               |
| 70                          | 346               |
| 80                          | 346               |
| 85                          | 346               |
| 65 Coke, per cent by weight | 14.4              |
|                             | Acidity           |
|                             | Per cent per cent |
| Aqueous distillate          | 15.5 0.4          |
| 70 Oil                      | 61.5 ---          |
| Coke, gas and loss          | 23.0 ---          |

There was produced by this operation 27.2% of motor fuel containing tar acids or 22% of motor fuel on an acid-free basis. There was concurrently produced 19.5% recycle stock which was

rerun to produce a total yield of 33% of tar acid-free motor fuel fraction.

As before, the crude motor fuel was treated with sulphuric acid and caustic soda, the tar acids separated from the alkali solution and fractionated into comparatively narrow boiling range cuts. All 25° C. fractions between 225° C. and 325° C. raised the induction period of the treated gasoline from 45 to above 240 minutes, the fraction from 275 to 300 having the greatest efficiency.

The following example gives data on the application of the process to the production of stable motor fuel from lignite tar.

|                                            |      |
|--------------------------------------------|------|
| Properties of lignite tar                  | 15   |
| Gravity °A. P. I.                          | 17.1 |
| Flash (Cleveland open cup) °F.             | 160  |
| Fire (Cleveland open cup) °F.              | 190  |
| Flash (Pensky-Martens) °F.                 | 125  |
| Viscosity, Furol@122° F., sec.             | 20   |
| Sulphur—per cent                           | 0.41 |
| Cold test °F.                              | 80   |
| B. S. & W.—per cent                        | 3.4  |
| Water (A. S. T. M. method 300.12)—per cent | 1.2  |
| Tar acids—per cent                         | 25.1 |
| Tar bases—per cent                         | 0.9  |
| 100 cc. A. S. T. M. distillation           |      |
| I. L. P., °F.                              | 210  |
| 5%                                         | 365  |
| 10                                         | 400  |
| 20                                         | 457  |
| 30                                         | 507  |
| 40                                         | 558  |
| 50                                         | 613  |
| 60                                         | 647  |
| 70                                         | 675  |
| 80                                         | 675  |
| 90                                         | 684  |
| E. P., °F.                                 | 693  |
| Per cent                                   | 40   |

|             |      |
|-------------|------|
| Over        | 96.0 |
| Coke by wt. | 4.3  |
| @ 400° F.   | 8.0  |
| @ 437° F.   | 14.5 |
| @ 572° F.   | 41.0 |

The tar was cracked under a pressure of 125 pounds per square inch and a temperature of 750° to 800° F., giving the following yields of products:

|                                    |      |
|------------------------------------|------|
| Gasoline fraction to 392° F.       | 33.5 |
| Intermediate gas oil recycle stock | 34.8 |
| Coke gas and loss                  | 30.1 |
| Water                              | 1.6  |
| Per cent                           | 50   |

The gas produced corresponded to 786 cubic feet per barrel of tar charged and the coke produced was in the amount of 69 pounds per barrel of charging stock. The gasoline and recycle stock had the properties shown in the following table:

| Properties                                       | Gasoline | Recycle stock |
|--------------------------------------------------|----------|---------------|
| Gravity °A. P. I.                                | 51.6     | 29.6          |
| Gum, mgs./100 cc. (copper dish)                  | 382      | 0.30          |
| Sulphur—percent                                  | 0.28     | 0.30          |
| Octane No.                                       | 65       |               |
| Tar acids—percent                                | 20.1     | 19.1          |
| Tar bases—percent                                | 0.7      | 0.6           |
| (100 cc. A. S. T. M. distillation) I. B. P., °F. | 128      | 404           |
| 5 percent                                        | 176      | 417           |
| 10                                               | 198      | 425           |
| 20                                               | 229      | 437           |
| 50                                               | 285      | 463           |
| 90                                               | 350      | 572           |
| E. P., °F.                                       | 392      | 644           |
| Percent over                                     |          | 98.5          |
| Percent bottoms                                  |          | 1.5           |

The gasoline was treated successively with 10% sulphuric acid and 10% sodium hydroxide to remove the tar bases and tar acids. After this treatment, the gasoline was further treated in 5 liquid phase at ordinary temperatures with ten pounds per barrel of 93% sulphuric acid, neutralized with caustic soda and rerun with fire and steam. The gasoline thus produced had the following properties:

|    |                               |      |
|----|-------------------------------|------|
| 10 | Gravity °A. P. I.             | 53.2 |
|    | Color, Saybolt                | 30   |
|    | Color stability*              | 25   |
|    | Mg. gum/100 cc. (copper dish) | 12   |
| 15 | Sulphur—per cent              | 0.13 |
|    | Octane number                 | 65   |

\*After four hours exposure to sunlight.

By treating the gasoline with only half the acid above shown, that is, 5 pounds per barrel instead 20 of 10, the color stability was found to be around 15 and the gum content in the neighborhood of 50 mgs. while the octane number was approximately 70 to 72%. The alkali solution of the tar acids was acidified and redistilled, the fraction 25 boiling from 240° to 300° C. being used as inhibiting material in an amount equal to 0.05%. The gasoline after the addition of this particular fraction of tar acids was found then to have substantially the same properties as the gasoline resulting from the 10 pound acid treatment in 30 respect to color, color stability, gums and sulphur while the octane number was still above 70%.

The foregoing specification and examples have 35 shown the value of the process in producing motor fuel which is effectively stabilized by the use of by-products of the overall operation. While the specification and examples are sufficient to accurately define the process and show its commercial advantages, neither is to be construed as imposing undue limitations thereon.

40 I claim as my invention:

1. A process for producing stabilized motor fuel distillate from tars containing phenolic compounds which comprises cracking the tar, separating phenolic substances from the resultant cracked distillate, distilling the separated phenolic substances and removing the cut thereof of highest inhibiting value, and adding such cut in small amount to the distillate as an inhibitor therefor.

50 2. A process for producing stabilized motor fuel distillate from tars containing phenolic compounds which comprises cracking the tar, separating phenolic substances from the resultant cracked distillate, distilling the separated phenolic substances and removing therefrom a cut boiling between 240° C. and 300° C., and adding such cut in small amount to the distillate as an inhibitor therefor.

55 3. A process for producing stabilized motor fuel distillate from tars containing phenolic compounds which comprises cracking the tar, extracting phenolic substances from the resultant cracked distillate, separating from the extract a select inhibitor fraction, and adding such fraction in small amount to the distillate as an inhibitor therefor.

4. In a process of stabilizing against gum formation, cracked hydrocarbon spirits of the type obtained by cracking hydrocarbons which produce substantial quantities of phenolic substances in the cracked gasoline, the steps of extracting the phenolic substances from the cracked gasoline and purifying the cracked gasoline by ordinary refinery treatment, separating by fractionation a portion of the phenolic extract having strong inhibiting properties and readding a 10 quantity of the phenolic substance to the refined cracked gasoline sufficient to substantially stabilize the same against gum formation.

5. In the treatment of cracked hydrocarbon distillates of the type obtained by cracking hydrocarbons which produce substantial quantities of phenolic substances in the cracked distillate, the steps of extracting the crude phenolic substances, converting the same to more highly effective inhibitor bodies, and readding the same to the 20 distillate in quantity sufficient to stabilize the distillate against gum formation.

6. A process for producing stabilized motor fuel distillate from hydrocarbon material containing phenolic compounds, which comprises 25 cracking the hydrocarbon material, extracting phenolic substances from resultant cracked products, separating from the extract a select inhibitor fraction, and adding such fraction in small amount to the overhead distillate of the 30 cracking as an inhibitor therefor.

7. A method for treating cracked hydrocarbon distillates obtained by cracking hydrocarbon materials which produce substantial quantities of phenolic substances in the cracked distillate, said 35 method comprising the steps of extracting phenolic substances from the distillate, separating from the extract a select inhibitor fraction, and re-adding such fraction to the distillate in sufficient amount to stabilize the distillate substantially 40 against gum formation.

8. A method for treating cracked hydrocarbon distillates obtained by cracking hydrocarbon materials which produce substantial quantities of phenolic substances in the cracked distillate, said 45 method comprising the steps of extracting phenolic substances from the distillate, producing from the resultant extract a material of high gum-inhibiting properties, and re-adding such material to the distillate in sufficient amount to stabilize the distillate substantially 50 against gum formation.

9. A method for treating cracked hydrocarbon distillates obtained by cracking hydrocarbon materials which produce substantial quantities of phenolic substances in the cracked distillate, said 55 method comprising the steps of extracting phenolic substances from the distillate, fractionating the resultant extract to separate therefrom a fraction having strong inhibiting properties, and re-adding such fraction to the distillate in sufficient amount to stabilize the distillate substantially 60 against gum formation.

JACQUE C. MORRELL.

65